# EUROPEAN PATENT SPECIFICATION

(11) **EP 1 920 079 B1**
(45) Date of publication and mention of the grant of the patent: **13.05.2009**
(21) Application number: 06789641.5
(22) Date of filing: 10.08.2006
(51) Int. Cl.: C22C 38/44, C22C 38/52, C22C 1/04, B22F 5/00, C22C 33/02

(54) **A MARAGING STEEL ARTICLE AND METHOD OF MANUFACTURE**
GEGENSTAND AUS MARAGING-STAHL UND ZUGEHÖRIGES HERSTELLUNGSVERFAHREN
ARTICLE EN ACIER MARAGING ET SON PROCÉDÉ DE FABRICATION

(30) Priority: 06.09.2005 US 218618
(43) Date of publication of application: 14.05.2008
(73) Proprietor: CRUCIBLE MATERIALS CORPORATION, Syracuse, NY 13201 (US)
(72) Inventor: MUHA, Joseph, F., Pittsburgh, PA 15237 (US); WOJCIESZYNSKI, Andrzej, L., Pittsburgh, PA 15241 (US); MCTIERNAN, Brian, J., Sewickley, PA 15143-1722 (US)
(74) Representative: Powell, Timothy John
(86) International application number: PCT/US2006/031111
(87) International publication number: WO 2007/030256

(56) References cited:
- EP-A- 0 648 852
- EP-A- 0 648 854
- GB-A- 1 243 382
- US-A- 5 482 531

## Description

### Field of the Invention

The invention relates to the manufacture of a maraging steel article with a specific composition using a powder metallurgy processing method. The steel as produced by practicing this invention, either in the AS-HIP condition or HIPed and hot worked condition, is appropriate for applications involving high temperatures or cyclic heating and cooling. The steel article of the invention has a hardness of less than 40 HRC after manufacturing and after solution heat treating, allowing the article to be machined. However, after the manufacture of the article and the subsequent maraging treatment, its hardness is greater than 45 HRC.

The applications for the steel article of the invention include processing of plastics or of liquid or hot solid metals, which include but are not limited to mold dies for the casting of liquid metals, mold dies for plastics, dies for forging other metals and dies for extruding. The cyclical heating and cooling of tools for these applications characterize these applications. This cyclical heating and cooling create sufficient stresses in the tool to cause thermal fatigue cracking, also known as heat checking. Different applications can tolerate different amounts of heat checking. For some products that require a high quality cosmetic appearance, the dies must be replaced after very limited heat checking has occurred. For other products that may not require this high quality cosmetic appearance, the dies can be used even with severe heat checking. In all cases, the majority of dies eventually fail and are replaced due to thermal fatigue cracking.

Existing hot work tool steels can suffice for the products with less stringent cosmetic requirements or shorter life time cycles. However, for product with a high cosmetic requirement, there is a need for a tool with a longer useful service life to satisfy the demands of the production practice.

### Prior Art

Tools are used in several applications involving the processing of hot metal. This metal can be in the liquid form, as in die-casting, or in the solid form, as in hot extrusion and hot forging. The useful life of all these tool materials is typically limited by thermal fatigue cracking. That is, as the process proceeds, more thermal fatigue cracks initiate on the surface of the tool, and existing thermal fatigue cracks grow. The die is replaced when the extent of thermal fatigue cracking renders the produced part as being of unacceptable quality. Requirements of steel used for high temperature applications include:

The material must have the capability to be heat-treated to greater than 45 HRC, which is the typical minimum working hardness for most tools of the prior art to maintain shape.

The material must also exhibit good high temperature strength. Fatigue cracking is related to the strength of the material. Therefore, a higher strength is one factor that can improve the resistance to thermal fatigue cracking.

Due to the die being exposed to high temperatures, softening of the die material can occur. This softening of the material will also decrease the strength of the material, making it more susceptible to thermal fatigue cracking. Therefore a tool material must exhibit good resistance to softening, also known as temper resistance.

Many of the tools used in the above operations are taken out of service due to the presence of thermal fatigue cracks. Thermal fatigue cracking has similarities to conventional fatigue cracking. However, in the case of thermal fatigue cracking, the stresses are introduced in the tool by cyclic heating and cooling. Therefore, it is important that material for such a tool exhibit good resistance to thermal fatigue cracking.

The thermal expansion of the tool during the heating and cooling cycle introduces stresses into the tool. Therefore, the material should have as low a coefficient of thermal expansion as possible or at minimum lower than the current materials in use.

Many tools are coated for resistance to erosion. Therefore, the die material must be capable of being coated by PVD (physical vapor deposition) or other relevant coating.

Although some applications may use the invention in the AS-HIP (as hot isostatically pressed condition, most applications will require the hot working of the material into smaller sections suitable for the customer. Therefore, the material must have good hot workability.

Several materials are currently used for hot work applications. The H series tool steels were developed for these applications, with the most common being the 5Cr hot work tool steels. This includes the steels known in the United States as H13 and H11. The H13 steel class is nominally in weight percent 0.38 carbon, 5.25 chromium, 1.25 molybdenum, 1.0 silicon and 1.0 vanadium. The H11 steel class is essentially the same as the H13 class but with weight percent 0.5 vanadium. For more severe applications, the H11 or H13 steel is typically processed using electro slag remelting (ESR) or vacuum arc remelting (VAR) methods.

Several variations of these 5 Cr tool steels have also been used. Among the most notable are H11 with lower silicon content for increased toughness. The other is a H11 with lower silicon and added molybdenum for improved temper resistance. Table 1 shows the nominal chemistries of some standard and some non-standard commercially available tool steels.

**Table 1**

| Nominal Chemical Composition of Selected Standard and Non Standard Hot Work Tool Steels | | | | | | | | |
|---|---|---|---|---|---|---|---|---|
| Alloy Designation | C | Si | Mn | Cr | Mo | V | Co | Fe |
| H10 | 0.32 | 0.25 | 0.30 | 3.00 | 2.80 | 0.50 | - | Bal. |
| H10A | 0.32 | 0.25 | 0.30 | 3.00 | 2.80 | 0.50 | 3.00 | Bal. |
| H11 | 0.40 | 1.00 | 0.25 | 5.30 | 1.60 | 0.40 | - | Bal. |
| H13 | 0.40 | 1.00 | 0.40 | 5.30 | 1.40 | 1.00 | - | Bal. |
| H19 | 0.45 | 0.40 | 0.40 | 4.50 | 3.00 | 2.00 | 4.50 | Bal. |
| Com. 1 | 0.36 | 0.20 | 0.50 | 5.25 | 1.65 | 0.50 | - | Bal. |
| Com. 2 | 0.36 | 0.20 | 0.50 | 5.00 | 2.35 | 0.60 | - | Bal. |
| Com. 3 | 0.36 | 0.20 | 0.40 | 5.20 | 1.95 | 0.60 | - | Bal. |
| 1.2367 | 0.38 | 0.40 | 0.40 | 5.00 | 3.00 | 0.60 | - | Bal. |
| Com. 4 | 0.38 | 0.20 | 0.25 | 5.00 | 3.00 | 0.60 | - | Bal. |

Among other materials which have been used in the past for hot work application are maraging steels. Most of them contain approximately 18% nickel and some titanium and obtain their hardness by precipitation of Ni-Mo and Ni-Ti particles. Many of these steels are aged using a relatively low temperature, typically less than 538°C (1000°F) which can limit the usefulness of the material when exposed to higher temperatures. Table 2 shows the nominal chemistries of some commercially available maraging steels.

**Table 2**

| Nominal Chemical Composition of Selected Maraging Steels | | | | | | | | | | | |
|---|---|---|---|---|---|---|---|---|---|---|---|
| Alloy | C | Si | Mn | Ni | Cr | Mo | Co | Cu | Ti | Al | B |
| Com. 1 | 0.008 | 0.15 | 0.05 | 17.5 | 0.10 | 4.90 | 11.00 | 0.20 | 0.13 | - | 0.003 |
| Com. 2 | 0.02 | 0.04 | 0.03 | 18.5 | 0.05 | 4.80 | 7.50 | - | 0.40 | 0.10 | 0.003 |
| Com. 3 | 0.02 | 0.05 | 0.03 | 18.5 | 0.10 | 4.90 | 9.00 | - | 0.60 | 0.10 | 0 |
| Com. 4 | 0.02 | - | - | 12.0 | - | 8.00 | 800 | - | 0.50 | 0.05 | - |

Some conventional maraging steels have been developed In the past with good thermal fatigue resistance and strength, but when produced by conventional methods have exhibited poor hot workability during processing from ingot stage to finished form. This poor hot workability results In either a defective final product or an insufficient yield (less than 50%) from ingot stage to finished stage to render the product commercially viable.
US-A-5,482,531, EP-A-0 648 852, GB-A-1 243 382 and EP-A-0 648 854 disclose maraging steel powder compositions and articles produced therefrom.

### SUMMARY OF THE INVENTION

The invention provides a new powder metallurgy produced maraging steel alloy article to be used as a tool for high temperature applications that satisfies the above-stated requirements. The article is fully dense and of prealloyed powder particles.

**Table 3**

| Chemistry Ranges for Alloy of invention | | | | | | | | |
|---|---|---|---|---|---|---|---|---|
| | C | Mn | Si | Cr | Mo | Ni | Co | S |
| Broad Range | 0.00-0.08 | 0.00-1.00 | 0.00-1.00 | 250-6.00 | 6.00-10.00 | 1.00-4.00 | 9.00-14.00 | 0.00-0.30 |
| Preferred Range | 0.00-0.05 | 0.10-0.50 | D.01D-0.50 | 4.00-5.75 | 7.00-9.00 | 1.50-3.00 | 10.00-1100 | 0.005-0.05 |
| More Preferred Range | 0.01-0.04 | 020-0.40 | 0.15-0.40 | 4.70-5.30 | 7.50-8.50 | 1.70-2.30 | 10.75-12.00 | 0.01-0.03 |

Hardening of the material is achieved by solution annealing and ageing, i.e. heating at a prescribed temperature for a prescribed length of time. This allows small precipitate particles to form, which in turn harden the low carbon martensitic structure of the material.

In the following, the importance of the individual alloying elements and their mutual interaction will be explained. All percentages related to the chemical composition in the specification and claims are in weight percent.

**Molybdenum** is a key element in the strengthening of this maraging steel, as the precipitate responsible for hardening the alloy is Fe₂Mo. It is also a key element in increasing the temper resistance of the alloy. Excessive quantities of molybdenum can allow the formation of detrimental delta ferrite.

**Cobalt** is required in a proper balance to prevent undesirable phases and to influence the aging process. Cobalt is an austenite former while preventing the formation of delta ferrite at high temperatures and has a minimal effect on the austenite to martensite transformation temperature. Cobalt also lowers the solubility of molybdenum in the martensitic matrix, thus making molybdenum more available for precipitation.

**Chromium** is desirable in some quantity for resistance to high temperature oxidation. Chromium in excessive quantity can result in the formation of delta ferrite.

**Nickel** also provides some benefit to oxidation resistance and is beneficial to mechanical properties. Excess nickel can cause the formation of austenite at typical service temperatures.

**Carbon** is not a critical element in the strengthening mechanism of this material.

**Silicon** is not a critical element in the properties of the alloy. Silicon may be used for deoxidizing during melting. It is a strong ferrite stabilizer.

**Manganese** is not critical for the properties of this alloy. It can be used to form manganese sulfide and therefore the content should be increased with increasing quantities of sulfur for enhanced machinability.

Sulfur may be present to promote machinability.

**Vanadium,** niobium, titanium, tungsten, zirconium, aluminum and other strong carbide and/or nitride formers are elements that are not desired and therefore should not exist in amounts above incidental impurity levels.

The alloy article of the invention is provided in the solution-annealed condition, which is performed by heating the material between 949°C and 1052°C (1740°F and 1925° F). Hardening by maraging is achieved by heating the material between 566°C and 738°C (1050°F and 1360°F).

### BRIEF DESCRIPTION OF THE DRAWINGS

Figure 1 is a graph showing the comparison of an alloy specimen within the composition limits of the invention produced by powder metallurgy and one produced by ESR with respect to ductility;

Figure 2 is a graph comparing the thermal fatigue resistance of a specimen in accordance with the invention and a specimen of H13 alloy; and

Figure 3 is a graph comparing hardness of a specimen in accordance with the invention and a specimen of H13 alloy.

### Performed Experiments and Specific Examples

Experiments were performed to determine various properties that were considered important to the successful performance of the alloy article of the invention. This included rapid strain tensile testing as a measure of hot workability, thermal fatigue cracking, temper resistance, tensile testing at room temperature and at 538°C (1000°F), determination of coefficient of thermal expansion and coating trials.

The following is the steel composition of the invention and H13 composition of the test specimens:

| Element | Maraging Alloy | ESR H13 |
|---|---|---|
| C | 0.019 | 0.40 |
| S | 0.011 | 0.002 |
| Mn | 0.32 | 0.27 |
| Si | 0.27 | 1.05 |
| Cr | 4.92 | 5.46 |
| Mo | 7.87 | 1.22 |
| V | <0.005 | 0.91 |
| Co | 11.17 | 0.04 |
| Ni | 1.89 | 0.15 |
| P | 0.015 | 0.009 |
| Al | <0.005 | 0.01 |
| Nb | <0.005 | <0.01 |
| Ti | <0.005 | <0.01 |
| W | 0.007 | <0.01 |
| O | 0.011 | 0.0017 |
| N | 0.023 | 0.005 |

### Rapid Strain Tensile Test

The rapid strain tensile testing was performed using the alloy article of the invention produced by powder metallurgy and electro slag remelted material of the same composition, In rapid strain testing, the specimens were heated by direct resistance heating. After achieving and equalizing at the desired test temperature, a load was applied to achieve a strain rate of 550 in / in / minute. This test is useful in simulating the conditions that exist during the hot working of the material.

Test temperatures were 982°C, 1038°C, 1093°C, 1148°C, 1177°C, 1204°C and 1232°C (1800°F, 1900°F, 2000°F, 2100°F, 2150°F, 2200°F and 2250°F). Figure 1 shows the reduction in area of the rapid strain rate tensile test for the specimens produced of the alloy of invention and the ESR material of the same composition. This clearly shows a substantial ductility advantage for the powder metallurgy material. The ductility of the ESR material was insufficient to permit hot working.

The rapid strain tests also are in agreement with experience on full size trials. Two full size compacts of the powder metallurgy alloy composition of the invention were produced and consolidated by hot isostatic pressing. Each compact was then processed to an intermediate size and then to a final size by hot rolling. Neither compact exhibited any hot working difficulties and the process yield was within the range of standard processing yield for other tool steels. By contrast, trials with full size ingots produced by ESR or other conventional methods exhibited poor hot workability during processing at the commercial steel making facility, resulting in process yields well below standard, including two heats that were scrapped entirely.

### Thermal Fatigue Resistance

Another important characteristic of hot work tool steels is thermal fatigue resistance. There are several tests available to measure thermal fatigue cracking, although none of these tests are a standard method (e.g. ASTM). Some testing is performed by heating a specimen to a high temperature using an induction coil for heating, then allowing the specimen to cool. This is performed over a number of cycles, with the specimen being evaluated periodically during the test. Another method involves testing a specimen with an internal cooling cavity for cooling water. This specimen is repeatedly immersed into a liquid aluminum bath. Again the cracking is rated periodically during the test.

The testing for the alloy of the invention was performed using a 12.7 mm (½") square by ~150 mm (6") long solid specimen produced by hot isostatic pressing and hot working. The test specimen can be tested simultaneously with up to five other specimens during the same procedure. The other specimen for this experiment was an ESR H13 material, which is the alloy most frequently used in aluminum die casting dies. The specimens were bolted to a holding plate affixed to the end of a mechanical arm which moved the specimens through the various stages of the test cycle. The arm immersed the specimens into molten aluminum to a depth of approximately 125 mm (5 inches) for 7 seconds. The specimens were then lifted out of the molten aluminum, moved to a position above a tank of water and then immersed into the water for 12 seconds. The specimens were then lifted out of the water, and the arm moved to a position above the molten aluminum for 5 seconds to dry the specimens. The cycle was then repeated.

During the trials, the specimens were periodically evaluated for thermal fatigue cracking, typically every 5,000 cycles. Two opposite faces of the specimens were cleaned using silicon carbide paper on a granite surface plate. The four cleaned corners of each specimen were then examined under a stereo microscope at a magnification of 90x. To avoid end effects, the examinations were conducted in an area 35 mm (1- 3/8") long, and which was located about 35 mm (1-3/8") from the bottom end of the specimens.

Each of the four corners was traversed along the 35 mm (1-3/8") length and the number of cracks and their lengths were recorded. There are numerous ways this data can be normalized, but experience with the test has shown little deviation in the ranking of the specimens. Therefore, the simple total number of cracks was divided by the number of corners (4) to obtain the number of cracks per corner. Figure 2 is a graphic representation of trial results of the powder metallurgy produced invention specimen versus the ESR H13 steel specimen. As previously discussed, the thermal fatigue cracking is the most frequent cause of tool failure. For this reason, it is believed that thermal fatigue testing provides the most important indication of the improved performance of the alloy of invention.

### Temper Resistance

A trial to determine the temper resistance of the alloy article of the invention was also performed. Both the PM alloy specimen of the invention and the H13 steel specimen were heat-treated to similar hardness levels, using typical heat-treat cycles for each material. An initial hardness was measured and recorded. Then the specimens were placed into a furnace at a temperature of 649°C (1200°F). One set of specimens was removed after 50 hours at temperature and the hardness level tested and recorded. Another set of specimens was removed after 100 hours at temperature and the hardness level tested and recorded. Figure 3 is a graphical representation of the hardness level as a function of hold time at 649°C (1200°F). It can be seen that the alloy of the invention has a superior temper resistance to H13 steel.

### Tensile Properties

Table 4 shows the results of tensile testing of the PM alloy article of the invention versus results for ESR H13 steel. Specimens tested were machined to a 6.35 mm (0.250") diameter with a 25.4 mm (1.00") gage length (4D). The results indicate that the alloy of invention has a higher yield and tensile strength at both room temperature and at 538°C (1000°F). This higher strength makes the alloy article of the invention less susceptible to thermal fatigue cracking,

**Table 4**

| Tensile Properties | | |
|---|---|---|
| | Invention Maraging Article (47 HRC) | ESR H13 Steel (45 HRC) |
| 72°F | | |
| UTS | 261 | 206 |
| YS | 207 | 185 |
| %El | 10 | 12 |
| RA | 25 | 55 |
| 1000°F | | |
| UTS | 161 | 145 |
| YS | 138 | 116 |
| %El | 23 | 15 |
| RA | 62 | 75 |

| | | |
|---|---|---|
| The °F temperatures in Table 4 are equivalent to Celsius temperatures in accordance with the conversion formula $°C temperature = \frac{5}{9} \left(°F temperature-32\right) .$ | | |

### Coefficient of Thermal Expansion

Thermal expansion is an important factor, both in the resistance of a tool to thermal fatigue cracking and in the final product quality of a tool. In both cases, a smaller coefficient of thermal expansion is desired. The significance of the lower coefficient of thermal expansion is that with less dimensional change, the tool Will be subjected to lower thermal stresses than a material with a greater dimensional change. The lower stresses present will thus render the tool more resistant to thermal fatigue cracking. The coefficient of thermal expansion was determined by the thermal dilatometric analysis (TDA) method. The coefficient of thermal expansion for the PM alloy article of the invention was determined to be 6.6 x 10⁻⁶ in. / in. °F over the temperature range of 22°C to 599°C (72°F to 1110°F). The ESR H13 die steel had a coefficient of 7.3 x 10⁻⁶ in. / in. / °F over the temperature range of 22°C to 599°C (72°F to 1110°F).

### Field Coating Trials

Field trials have shown the PM invention alloy article is easily coated with either a physical vapor deposition (PVD) process or chemical vapor deposition (CVD) which employs a higher temperature than the PVD process. The alloy article of the invention was coated with TiN, TiAIN and CrN PVD coatings. The coatings were deposited at a high deposition rate at a temperature range of 399°C to 454°C (750-850°F) for both the article of the invention and ESR H13 steel. Unlike many other maraging steels, this temperature is well bellow the aging temperature for the alloy article of the invention.

Similarly, the coating was deposited using a chemical vapor deposition process on both the alloy article of the invention and conventional tool steel material. Conventional tool steels are not well suited for CVD, as the coating process typically takes place at a temperature above the critical temperature of these alloy. The advantage provided by the article of the invention is that the CVD process results in the required heat treatment, namely solution annealing. After coating, the invention article requires only a single aging treatment. The nature of the maraging process is such that the dimensional changes of the tool are very minimal, allowing for good adherence of the coating to the substrate.

## Claims

1. A fully dense, powder-metallurgy produced steel alloy article of prealloyed powder having a managing microstructure for use as a tool for high temperature applications comprising, in weight percent:
C 0.08 max., Mn 1.0 max., Si 1.0 max., Cr 2.5 - 6.0, Mo 6.0-10.0, Ni 1.0 - 4.0, Co 9.0 - 14.0, sulfur up to 0.3 and balance iron and incidental impurities;
said article as-produced having a hardness of less than 40 HCR to provide machinability; and
thereafter said article upon maraging heat treatment having a hardness greater than 45 HRC.

2. The article of claim 1, comprising, in weight percent, C 0.05 max., Mn 0.1 to 0.05, Si 0.01 to 0.5, Cr 4 to 5.75, Mo 7 to 9, Ni 1.5 to 3, Co 10 ' 0.5 to 13, S 0.005 to 0.5 and balance iron and incidental impurities.

3. The alloy article of claims 1 comprising, in weight percent, C 0.01 to 0.04, Mn 0.2 to 0.4, Si 0.15 to 0.4, Cr 4.7 to 5.3, Mo 7.5 to 8.5, Ni 1.7 to 2.3, Co 10.75 to 12, S 0.01 to 0.03 and balance iron and incidental impurities.

4. The article of claims 1, 2 or 3, wherein said article is in the form of a die.

5. The article of claims 1, 2 or 3, wherein said article is in the form of a container for liquid metal.

6. A method for producing an article for use In processing of hot metal comprising:
compacting prealloyed powder of a maraging steal to produce a fully dense article having a hardness of less than 40 HRC to provide machinability;
thereafter maraging heat treating said article to achieve a hardness greater than 45 HRC; and
said prealloyed powder comprising, in weight percent C 0.08. max., Mn 1.0 max., Si 1.0 max., Cr 2.5 - 6.0, Mo 6.0 -10.0, Ni 1.0 - 4.0, Co 9.0 -14.0, sulfur up to 0.3 and balance iron and incidental impurities.

7. The methods of claim 6, wherein said prealloyed powder comprises, in weight percent, C 0.05 max., Mn 0.1 to 0.5, Si 0.01 to 0.5, Cr 4 to 5.75, Mo 7 to 9, Ni 1.5 to 3, Co 10 to 13, S 0.005 to 0.05 and balance iron and incidental impurities.

8. The method of claim 6, wherein said prealloyed powder comprises, in weight percent, C 0.01 to 0.04, Mn 0.2 to 0.4, Si 0.15 to 0.4, Cr 4.7 to 5.3, Mo 7.5 to 8.5, Ni 1.7 to 2.3, Co 10.75 to 12, S 0.01 to -0.03 and balance iron and incidental impurities.

9. The method of claim 6, 7 or 8, wherein maraging heat treatment is performed at temperatures within a range of 540 to 700 degrees C.

## Patentansprüche

1. Vollständig dichter, durch Pulvermetallurgie hergestellter Stahllegierungsgegenstand aus einem vorlegierten Pulver mit Maraging-Mikrostruktur zur Verwendung als Werkzeug für Hochtemperaturanwendungen, umfassend - in Gewichtsprozent:
max. 0,08 C, max. 1,0 Mn, max. 1,0 Si, 2,5-6,0 Cr, 6,0-10,0 Mo, 1,0-4,0 Ni, 9,0-14,0 Co, Schwefel bis zu 0,3 und zum Rest Eisen und beiläufige Verunreinigungen;
wobei der Gegenstand nach der Herstellung eine Härte von weniger als 40 HRC zur Bereitstellung von Spanbarkeit aufweist und der Gegenstand dann nach einer Maraging-Wärmebehandlung eine Härte von größer als 45 HRC aufweist.

2. Gegenstand nach Anspruch 1, der - in Gewichtsprozent - max. 0,05 C, 0,1 bis 0,05 Mn, 0,01 bis 0,5 Si, 4 bis 5,75 Cr, 7 bis 9 Mo, 1,5 bis 3 Ni, 10 bis 13 Co, 0,005 bis 0,5 S und zum Rest Eisen und beiläufige Verunreinigungen umfasst.

3. Legierungsgegenstand nach Anspruch 1, der - in Gewichtsprozent - 0,01 bis 0,04 C, 0,2 bis 0,4 Mn, 0,15 bis 0,4 Si, 4,7 bis 5,3 Cr, 7,5 bis 8,5 Mo, 1,7 bis 2,3 Ni, 10,75 bis 12 Co, 0,01 bis 0,03 S und zum Rest Eisen und beiläufige Verunreinigungen umfasst.

4. Gegenstand nach Anspruch 1, 2 oder 3, wobei der Gegenstand die Form eines Formwerkzeugs aufweist.

5. Gegenstand nach Anspruch 1, 2 oder 3, wobei der Gegenstand die Form eines Behälters für ein flüssiges Metall aufweist.

6. Verfahren zur Herstellung eines Gegenstands zur Verwendung bei der Verarbeitung eines heißen Metalls, umfassend:
das Kompaktieren eines vorlegierten Pulvers eines Maraging-Stahls zur Herstellung eines vollständig dichten Gegenstands, der eine Härte von weniger als 40 HRC zur Bereitstellung von Spanbarkeit aufweist;
eine nachfolgende Maraging-Wärmebehandlung des Gegenstands, um eine Härte von größer als 45 HRC zu erreichen; und
wobei das vorlegierte Pulver - in Gewichtsprozent - max. 0,08 C, max. 1,0 Mn, max. 1,0 Si, 2,5-6,0 Cr, 6,0-10,0 Mo, 1,0-4,0 Ni, 9,0-14,0 Co, Schwefel bis zu 0,3 und zum Rest Eisen und beiläufige Verunreinigungen umfasst.

7. Verfahren nach Anspruch 6, wobei das vorlegierte Pulver - in Gewichtsprozent - max. 0,05 C, 0,1 bis 0,5 Mn, 0,01 bis 0,5 Si, 4 bis 5,75 Cr, 7 bis 9 Mo, 1,5 bis 3 Ni, 10 bis 13 Co, 0,005 bis 0,05 S und zum Rest Eisen und beiläufige Verunreinigungen umfasst.

8. Verfahren nach Anspruch 6, wobei das vorlegierte Pulver - in Gewichtsprozent - 0,01 bis 0,04 C, 0,2 bis 0,4 Mn, 0,15 bis 0,4 Si, 4,7 bis 5,3 Cr, 7,5 bis 8,5 Mo, 1,7 bis 2,3 Ni, 10,75 bis 12 Co, 0,01 bis 0,03 S und zum Rest Eisen und beiläufige Verunreinigungen umfasst.

9. Verfahren nach Anspruch 7, 8 oder 9, wobei die Maraging-Wärmebehandlung bei Temperaturen innerhalb eines Bereichs von 540 bis 734 °C durchgeführt wird.

## Revendications

1. Article en alliage d'acier très dense (« fully dense ») produit par métallurgie des poudres, constitué d'une poudre préalliée, présentant une microstructure maraging pour une utilisation en tant qu'outil pour des applications à haute température comprenant, en pourcentage en poids :
C, 0,08 max., Mn, 1,0 max., Si, 1,0 max., Cr, 2,5 à 6,0, Mo, 6,0 à 10,0, Ni, 1,0 à 4,0, Co, 9,0 à 14,0, du soufre jusqu'à 0,3 et le reste étant du fer et des impuretés non intentionnelles ;
ledit article tel que produit présentant une dureté inférieure à 40 HRC pour fournir une aptitude à l'usinage ; et
ledit article, par la suite, lors du traitement thermique de maraging, présentant une dureté supérieure à 45 HRC.

2. Article selon la revendication 1, comprenant, en pourcentage en poids, C, 0,05 max., Mn, 0,1 à 0,05, Si, 0,01 à 0,5, Cr, 4 à 5, 75, Mo, 7 à 9, Ni, 1,5 à 3, Co, 10 à 13, S, 0,005 à 0,5 et le reste étant du fer et des impuretés non intentionnelles.

3. Article en alliage selon la revendication 1, comprenant, en pourcentage en poids, C, 0,01 à 0,04, Mn, 0,2 à 0,4, Si, 0,15 à 0,4, Cr, 4,7 à 5,3, Mo, 7,5 à 8,5, Ni, 1,7 à 2,3, Co, 10,75 à 12, S, 0,01 à 0,03 et le reste étant du fer et des impuretés non intentionnelles.

4. Article selon la revendication 1, 2 ou 3, dans lequel ledit article se présente sous la forme d'une matrice.

5. Article selon la revendication 1, 2 ou 3, dans lequel ledit article se présente sous la forme d'un récipient pour un métal liquide.

6. Procédé de préparation d'un article pour une utilisation dans le traitement d'un métal chaud, comprenant :
la compression d'une poudre préalliée d'un acier maraging afin de préparer un article, très dense présentant une dureté inférieure à 40 HRC pour fournir une aptitude à l'usinage ;
par la suite, le traitement thermique de maraging audit article afin d'obtenir une dureté supérieure à 45 HRC ; et
ladite poudre préalliée comprenant, en pourcentage en poids, C, 0,08 max., Mn, 1,0 max., Si, 1,0 max., Cr, 2,5 à 6,0, Mo, 6,0 à 10,0, Ni, 1,0 à 4,0, Co, 9,0 à 14,0, du soufre jusqu'à 0,3 et le reste étant du fer et des impuretés non intentionnelles.

7. Procédé selon la revendication 6, dans lequel ladite poudre préalliée comprend, en pourcentage en poids, C, 0,05 max., Mn, 0,1 à 0,5, Si, 0, 01 à 0,5, Cr, 4 à 5,75, Mo, 7 à 9, Ni, 1,5 à 3, Co, 10 à 13, S, 0,005 à 0,05 et le reste étant du fer et des impuretés non intentionnelles.

8. Procédé selon la revendication 6, dans lequel ladite poudre préalliée comprend, en pourcentage en poids, C, 0,01 à 0,04, Mn, 0,2 à 0,4, Si, 0,15 à 0,4, Cr, 4,7 à 5,3, Mo, 7,5 à 8,5, Ni, 1,7 à 2, 3, Co, 10, 75 à 12, S, 0,01 à 0,03 et le reste étant du fer et des impuretés non intentionnelles.

9. Procédé selon la revendication 7, 8 ou 9, dans lequel le traitement thermique de maraging est réalisé à des températures dans la gamme de 540 à 734 degrés C.
